

## UNITED STATES PATENT OFFICE

2,316,248

## ISOMERIZATION OF PARAFFINS

Vladimir N. Ipatieff and Herman Pines, Chicago,  
Ill., assignors to Universal Oil Products Company,  
Chicago, Ill., a corporation of Delaware

No Drawing. Application January 12, 1940,  
Serial No. 313,527

15 Claims. (Cl. 260—683.5)

This invention relates to the treatment of paraffins to produce more highly branched hydrocarbons and particularly to the treatment of butane of normal or straight chain structure.

More specifically the invention is concerned with a process whereby normal butane is converted into isobutane, the process involving the use of special catalysts and particular conditions of operation which favor isomerization so that the iso-compound is produced in relatively high yield.

Since the invention is concerned principally with the two 4-carbon atom paraffin hydrocarbons and their transformation, one into the other, the following table is introduced to indicate the structure and the principal physical characteristics of these two compounds:

*Properties of butanes*

| Name       | Structure                                                                                                | B. P., °C. | Critical temperature, °C. | Critical pressure, atms. |
|------------|----------------------------------------------------------------------------------------------------------|------------|---------------------------|--------------------------|
| n-Butane   | CH <sub>3</sub> CH <sub>2</sub> CH <sub>2</sub> CH <sub>3</sub>                                          | +0.5       | 151                       | 36                       |
| Iso-butane | $  \begin{array}{c}  \text{CH}_3 \\    \\  \text{CH} - \text{CH}_2 \\    \\  \text{CH}_3  \end{array}  $ | -10.5      | 134.5                     | 37                       |

Butanes are produced in considerable quantities in the oil refining industry. They occur in substantial amounts in natural gases (in which the normal compound usually predominates), in refinery gases which are evolved from crude petroleum storage tanks, and in the primary distillation of crudes, and they are also present in considerable percentages in the gases produced incidental to cracking heavy petroleum fractions for the production of gasoline. In the case of cracked gas mixtures the relative proportions of iso- and normal-butanes vary, but the ratio of the iso- to the normal-compound is as a rule considerably higher than in natural gas.

Butanes may be considered as more or less marginal compounds in respect to their desirability in ordinary gasoline, that is, a certain percentage of them is essential for sufficient vapor pressure to insure ease in starting, while an excess tends to produce vapor lock. For these reasons the total percentage of 4-carbon atom hydrocarbons is commonly adjusted in conjunction with the boiling range and vapor pressure of the other gasoline components to produce a gasoline of desirable starting characteristics according to seasonal demands.

The butanes at the present time bear a further important relationship to oil refining in that their excess production is being utilized as a source of gasoline either by ordinary thermal cracking or by special catalytic dehydrogenation processes followed by polymerization in which catalysts may or may not be used. Investigations have shown that isobutane is considerably more amenable to cracking and dehydrogenation, both with and without catalysts, than the normal compound. Considering the corresponding monoolefins, the normal butenes are considerably more difficult to polymerize, either thermally or catalytically, than isobutene, and it is found that also the octenes representing the dimers of isobutene are of a higher antiknock value than those from n-butenes which holds also for the octanes produced by hydrogenation. It is, therefore, of considerable importance at the present time to convert as much as possible of the normal butane production into isobutane, and the present invention is especially concerned with a process for accomplishing this object.

In one specific embodiment the present invention comprises a process for producing isobutane from normal butane which comprises contacting said normal butane with a composite of substantially anhydrous chlorides of aluminum and copper and a porous adsorbent in the presence of small but definite quantities of hydrogen halide and under isomerizing conditions of temperature and pressure.

We have determined by the use of the class of catalysts mentioned, and particularly by the concurrent use of considerable superatmospheric pressure, normal butane may be converted into approximately 30-60% of isobutane per pass. Practical yields of isobutane are obtainable at temperatures within the approximate range of 50-350° C. under pressures of the order of 1 to 200 atmospheres and preferably of 10 to 200 atmospheres at temperatures of 150° C. and higher. Besides depressing the volatilization of aluminum chloride from such catalysts, pressure tends also to diminish numerous undesirable side reactions which would result in the formation of hydrogen and of low molecular weight hydrocarbons, so that the reaction proceeds more or less in one direction until an equilibrium is established.

There are several alternative catalysts consisting of aluminum chloride and copper chloride on inert carrying materials which may be employed in effecting the isomerization of normal butane to isobutane; and while they may be used more or less interchangeably, some are more

effective than others, and accordingly it is not intended to infer that they are definitely equivalent. Extensive experiments have indicated that best results are obtained when a minor percentage of a hydrogen halide, usually in the approximate range of 0.5-10% by volume of the butane, is present in the reactions and the necessary amount of hydrogen halide may be introduced directly or produced in situ by small amounts of water or steam, which cause a certain amount of hydrolysis of the substantially anhydrous chlorides.

One of the essential features of the present invention is the use of active aluminum chloride diluted by copper chloride in conjunction with porous granular supports. This use of supports facilitates vapor phase operations at temperatures above the sublimation point of aluminum chloride and apparently in some instances seems to lessen the tendency to the formation of sludges consisting of complex addition compounds so that the life of the catalyst extended materially.

When granular aluminum chloride is employed alone in hydrocarbon reactions, it soon tends to agglomerate on account of the formation of adhesive sludge-like materials so that violent agitation is necessary to maintain contact of the catalyst with the reacting hydrocarbons. Among supporting materials which we have now shown to have practical value as carriers may be mentioned activated carbon, pumice, various types of fuller's earths and clays, particularly those of the montmorillonite or bentonite types, either raw or acid treated, diatomaceous and infusorial earths, kieselguhr, silica-alumina composites, unglazed porcelain, firebrick, and, in general, refractory porous substances which have substantially no reactivity with the anhydrous chlorides. It happens frequently that one type of support is better than others, depending upon the ratios of chlorides and support found experimentally to be the best for the furtherance of a particular isomerizing reaction so that it is not to be inferred that the supports can at all times be used interchangeably.

A property of anhydrous aluminum chloride which must be taken into account is its tendency to sublime at a temperature of approximately 180° C., so that if it is employed at temperatures above this point it must ordinarily be injected or sublimed into the reaction zone.

In the process of the present invention in which the mixture of aluminum chloride and cupric chloride employed is strongly adsorbed by granular material, the enumerated disadvantages of unsupported aluminum chloride are overcome to a large extent since the tendency of aluminum chloride to volatilize is particularly counteracted by the adsorbent action of the supports employed, and these supports further act to adsorb and retain some of the viscous addition compounds and prevent the composite catalyst granules from adhering to form large agglomerates.

A general method of preparation of the types of granules whose use in butane isomerization characterizes the present invention consists in precipitating cupric oxide upon a carrier, for example firebrick, converting the cupric oxide to copper chloride and compositing the resultant granular material with aluminum chloride. This procedure may be carried out by impregnating the carrier with an aqueous solution of cupric chloride, then adding a basic precipitant as ammonium hydroxide to form finely divided cupric oxide or copper hydroxide, after which the aqueous solution is evaporated to leave the cupric

oxide deposited upon the carrier. The carrier and supported cupric oxide may then be dried preferably in a stream of an inert gas as nitrogen at approximately 200° C. A slow stream of hydrogen chloride is then passed over the dried granular material as its temperature is increased slowly from approximately 200 to 400° C. during which the material changes color from dark blue to dark brown, characteristic of anhydrous cupric chloride.

The resultant granular composite of carrier and copper chloride is then mixed with the desired quantity of anhydrous aluminum chloride and heated in a pressure vessel at approximately 250° C. preferably in the presence of hydrogen chloride and under approximately 25 atmospheres pressure of hydrogen or of another inert gas. After treating the granules of copper chloride and carrier with aluminum chloride, the composite obtained appears dry and the aluminum chloride has apparently disappeared although its presence in the pores and on the surface of the composite is evident by the violent reaction of the granules with water and their catalytic activity in organic reactions. This procedure is typical of the preparation of any number of similar catalytic materials using different proportions of metal chlorides on the supports herein mentioned.

The addition of copper chloride to aluminum chloride used for preparing a supported isomerization catalyst increases the isomerizing activity and life over that obtainable with similar catalytic material consisting of aluminum chloride only deposited upon substantially inert supports. In the presence of the supported aluminum chloride-copper chloride catalyst there is also relatively small formation of propane and pentane from butane by side reactions.

Owing to the adsorptive properties of the supports, catalysts of the above character may be employed in isomerizing normal butane with substantially no tendency for the original particles to run together due to the formation of intermediate sludge-like products, so that much larger quantities of material may be treated before the catalyst has lost its activity. Another advantage resides in the fact that the adsorbed halides will remain in place without volatilization at considerably higher temperatures than the normal sublimation point of aluminum chloride when normal butane is passed over a stationary granular bed of the catalyst composite.

The term "activated carbon" as used in the present specification is intended to include any type of prepared carbon or carbonaceous material which is more or less granular and possessed of good porosity and structural strength and which has been prepared by general steps involving the leaching of adsorbed material from granular residual carbonaceous materials such as wood char and various varieties of coke by mineral acids and by the controlled heating, preferably under vacuum, to expel adsorbed liquids and gases. It is recognized that various forms of active granular chars will vary considerably in adsorptive capacity and, therefore, the properties of catalysts prepared when using them in accordance with the present invention will vary both in respect to the amount of aluminum and copper chlorides which they are able to adsorb and in respect to the periods of service in which they are able to maintain a practical activity in different organic reactions.

The present butane isomerization process may

be operated under batch or continuous conditions and either in liquid, mixed, or vapor-phase as may be desirable or expedient in view of the particular combination chosen. A simple method of operation consists in adding 5 to 10 percent of a granular catalyst composite to a treating vessel containing hydrocarbons and provided with a mechanical agitating device of some description. It is preferable to employ a treater which can be sealed from atmospheric contact and which can be operated under pressure if necessary. The solid catalyst is then kept in suspension by moderate agitation while introducing a slow stream of hydrogen chloride, or other hydrogen halide. Addition of hydrogen to the reaction mixture also tends to decrease sludge formation and prolong the life of the catalyst composite employed in isomerization reactions.

In another type of operation which accelerates the rate of isomerization, the hydrocarbon mixture may be kept at its boiling point by moderate heating under reflux conditions with the granular catalyst maintained in suspension by the ebullition, while the hydrogen halide is added in a slow stream. In this type of operation any desired superatmospheric pressure may be employed to permit the use of any desired temperature. In the case of a supported aluminum chloride-copper chloride composite, the necessary amount of hydrogen chloride may be generated by adding a small amount of water or steam which causes hydrolysis.

Vapor phase isomerization operations may be conducted by passing vapors of hydrocarbons mixed with a small amount of hydrogen chloride over catalyst composites in the form of granules or pellets which are contained in treating chambers or reactors. Addition of hydrogen to such reaction mixtures has a beneficial effect similar to that observed during its use in batch operations.

While the catalyst and process of this invention are particularly useful in isomerizing normal butane into isobutane, they may be used also for isomerizing normally liquid paraffins into more branched isomeric paraffins under conditions of temperature, pressure, and time found to be optimum for the isomerization of the hydrocarbons or hydrocarbon mixtures undergoing treatment.

The following example is introduced as characteristic of the practical operation of the present process although not with the intention of limiting the scope of the invention in exact correspondence with the numerical data since some latitude is possible in the proportions of adsorbent, aluminum chloride, and copper chloride; and temperatures and pressures may also be varied within the limits already specified. These variations may be considerable in the case of gas mixtures in which the normal butane content varies over relatively wide ranges.

#### Example

A solution containing 3 parts by weight of copper chloride in 300 parts by weight of water was added to 90 parts by weight of 6-10 mesh crushed firebrick and then ammonium hydroxide solution was added to produce a precipitate of copper hydroxide. Afterward the water was evaporated slowly over a water bath leaving a composite of firebrick and cupric oxide which was dried in a glass tube at 200° C. in a stream of nitrogen. A slow stream of hydrogen chloride was then passed over the dried granular composite

while the temperature was increased from 200 to 400° C. over a period of 20 hours during which a dark brown color characteristic of anhydrous cupric chloride developed in the granular composite. The firebrick containing cupric chloride was next mixed with 50 parts by weight of aluminum chloride and heated in an autoclave at 250° C. in the presence of 10 parts by weight of hydrogen chloride and under a hydrogen pressure of 25 atmospheres. After this treatment for two hours a granular composite was obtained containing 30 parts by weight of aluminum chloride, 3 parts by weight of cupric chloride, and 70 parts by weight of firebrick.

Normal butane containing 4% by volume of hydrogen chloride was passed through a tube containing 47 parts by weight (75 volumes) of the above described granular composite at 200° C. under a pressure of 45 atmospheres. The normal butane which had been saturated previously with hydrogen under 45 atmospheres pressure was charged at the rate of 1.1 volumes per hour per volume of reactor space containing the granular composite catalyst. It was found that 4,850 volumes of liquid isobutane and 610 volumes of pentane were formed from 14,200 volumes of normal butane in the presence of the 75 volumes of granular composite catalyst before the isomerization decreased to 15% per pass. During the run, the average molar composition of the exit gases per pass was 4.7% propane, 34.2% isobutane, 56.8% normal butane, and 4.3% pentanes. A similar catalyst but without copper chloride under similar conditions produced 3,570 volumes of liquid isobutane and 440 volumes of pentanes from 11,000 volumes of normal butane before the percentage isomerization decreased to 15% per pass.

The character of the present invention and its novelty and utility in producing isobutane from normal butane in the presence of supported aluminum chloride-copper chloride composites can be seen from the preceding specification and numerical data presented although neither section is intended to unduly limit its generally broad scope.

We claim as our invention:

1. A process for the isomerization of paraffin hydrocarbons to produce therefrom substantial yields of compounds more highly branched than the materials subjected to treatment which comprises subjecting said hydrocarbons mixed with a hydrogen halide to contact with a granular composite of substantially anhydrous chlorides of aluminum and copper and a relatively inert adsorbent under isomerizing conditions of temperature and pressure.
2. A process for the isomerization of normally liquid paraffin hydrocarbons to produce therefrom substantial yields of compounds more highly branched than the materials subjected to treatment which comprises subjecting said hydrocarbons mixed with a hydrogen halide to contact with a granular composite of substantially anhydrous chlorides of aluminum and copper and a relatively inert adsorbent under isomerizing conditions of temperature and pressure.
3. A process for the isomerization of normal butane to produce therefrom substantial yields of isobutane which comprises subjecting said normal butane mixed with a hydrogen halide to contact with a granular composite of substantially anhydrous chlorides of aluminum and copper and a relatively inert adsorbent under isomerizing conditions of temperature and pressure.

3. A process for the isomerization of normal butane to produce therefrom substantial yields of isobutane which comprises subjecting said normal butane mixed with a hydrogen halide to contact with a granular composite of substantially anhydrous chlorides of aluminum and copper and a relatively inert adsorbent under isomerizing conditions of temperature and pressure.

4. A process for the isomerization of normal butane to produce therefrom substantial yields of

isobutane which comprises subjecting said normal butane mixed with a hydrogen halide to contact with a granular composite of substantially anhydrous chlorides of aluminum and copper and a relatively inert siliceous adsorbent.

5. A process for the isomerization of normal butane to produce therefrom substantial yields of isobutane which comprises subjecting said normal butane mixed with a hydrogen halide to contact at a temperature within the approximate range of 50-350° C. with a granular composite of substantially anhydrous chlorides of aluminum and copper and a relatively inert adsorbent.

6. A process for the isomerization of normal butane to produce therefrom substantial yields of isobutane which comprises subjecting said normal butane mixed with a hydrogen halide to contact at a temperature within the approximate range of 50-350° C. with a granular composite of substantially anhydrous chlorides of aluminum and copper and a relatively inert siliceous adsorbent.

7. A process for the isomerization of normal butane to produce therefrom substantial yields of isobutane which comprises subjecting said normal butane mixed with a hydrogen halide to contact at a temperature within the approximate range of 50-350° C. under a pressure of a substantially inert gas from substantially atmospheric to approximately 200 atmospheres with a granular composite comprising essentially anhydrous chlorides of aluminum and copper and a relatively inert adsorbent.

8. A process for the isomerization of normal butane to produce therefrom substantial yields of isobutane which comprises subjecting said normal butane mixed with a hydrogen halide to contact at a temperature within the approximate range of 50-350° C. under a pressure of an inert gas from substantially atmospheric to approximately 200 atmospheres with a granular composite comprising essentially anhydrous chlorides of aluminum and copper and a relatively inert siliceous adsorbent.

9. A process for the isomerization of normal butane to produce therefrom substantial yields of isobutane which comprises subjecting said normal butane mixed with a hydrogen halide to contact at a temperature within the approximate range of 50-350° C. under a pressure of hydrogen from substantially atmospheric to approximately 200 atmospheres with a granular composite comprising essentially anhydrous chlorides of aluminum and copper and a relatively inert adsorbent.

10. A process for the isomerization of normal butane to produce therefrom substantial yields of isobutane which comprises subjecting said normal butane mixed with a hydrogen halide to contact at a temperature within the approximate range of 50-350° C. under a pressure of hydrogen from substantially atmospheric to approximately 200 atmospheres with a granular composite comprising essentially anhydrous chlorides of aluminum and copper and a relatively inert siliceous adsorbent.

11. A process for the isomerization of normal butane to produce therefrom substantial yields of isobutane which comprises subjecting said normal butane mixed with a hydrogen halide to contact at a temperature within the approximate range of 50-350° C. under a pressure of hydrogen from substantially atmospheric to approximately 200 atmospheres with a granular composite consisting of activated carbon and substantially anhydrous chlorides of aluminum and copper.

12. A process for the isomerization of normal butane to produce therefrom substantial yields of isobutane which comprises subjecting said normal butane mixed with a hydrogen halide to contact at a temperature within the approximate range of 50-350° C. under a pressure of hydrogen from substantially atmospheric to approximately 200 atmospheres with a granular composite of crushed firebrick and substantially anhydrous chlorides of aluminum and copper.

13. A process for the isomerization of normal butane to produce therefrom substantial yields of isobutane which comprises subjecting said normal butane mixed with a hydrogen halide to contact at a temperature within the approximate range of 50-350° C. under a pressure of hydrogen from substantially atmospheric to approximately 200 atmospheres with a granular composite of diatomaceous earth and substantially anhydrous chlorides of aluminum and copper.

14. A process for isomerizing paraffin hydrocarbons which comprises contacting the paraffins under isomerizing conditions with a solid catalyst comprising aluminum chloride and copper chloride.

15. A process for producing isobutane which comprises contacting normal butane under isomerizing conditions with a solid catalyst comprising aluminum chloride and copper chloride.

VLADIMIR N. IPATIEFF.  
HERMAN PINES.